

# UNITED STATES PATENT OFFICE.

WILLIAM E. RUDER, OF SCHENECTADY, NEW YORK, ASSIGNOR TO GENERAL ELECTRIC COMPANY, A CORPORATION OF NEW YORK.

## PROCESS OF MAKING MAGNETIC MATERIAL.

1,201,633.

Specification of Letters Patent. Patented Oct. 17, 1916.

No Drawing.

Application filed April 6, 1916. Serial No. 89,411.

To all whom it may concern:

Be it known that I, WILLIAM E. RUDER, a citizen of the United States, residing at Schenectady, in the county of Schenectady, State of New York, have invented certain new and useful Improvements in the Process of Making Magnetic Material, of which the following is a specification.

My invention has reference to the conversion of ordinary unalloyed, oxygenous iron, and especially of commercially pure unalloyed, oxygenous iron, particularly in sheet form, to a new state in which this material exhibits improved magnetic qualities which are especially useful in transformer cores, and in cores or frames for other alternating current apparatus.

I have heretofore discovered that the hysteresis of silicon steel is greatly reduced by the coalescence of the normal small grains of the material, which the unaided eye cannot resolve, into grains that are large enough to appear separated to the unaided eye, and by removing from the material all impurities such as sulfur, phosphorus and carbon, but particularly the oxygen which is combined with or is occluded in the material, so that all oxidulated compounds in the steel become reduced and the new material becomes practically non-oxygenous. For the realization of this discovery I have invented a process, and have secured a Patent, No. 1,110,010, dated September 8, 1914. The specific process described in my aforesaid patent consists in subjecting the silicon steel to a high temperature either in a partial vacuum (under a gas pressure at or below the dissociation pressures of the oxids in the material for the prevailing temperature) or in an atmosphere of a reducing gas such as hydrogen; and in the said patent I have described and illustrated suitable apparatus for practising the said invention.

Now, the low hysteresis property imparted to silicon steel by the process described in my aforesaid patent can also be imparted to ordinary unalloyed, oxygenous iron and particularly to commercially pure iron, such as is produced by the open hearth—or Bessemer—or crucible process, and, in addition, a valuable property not possessed by silicon steel can be imparted to such ordinary iron, namely, exceptionally high permeability. These results can be obtained by performing upon such ordinary iron substantially the

same acts which result in the improvement of silicon steel in accordance with my aforesaid patent. I have also discovered that the property of non-aging, which heretofore was believed to be dependent upon the presence of silicon or other alloying materials in the iron, can by the same acts, also be imparted to unalloyed, oxygenous iron. The new product is practically free of sulfur, phosphorus, carbon and oxygen and it shows substantially the same large grains as the improved silicon steel. In addition to this the new raw material used, namely, either ordinary or commercially pure unalloyed, oxygenous iron, being far less brittle and much softer than silicon steel, can be produced and subjected to the process in thinner sheets, which is a considerable advantage, particularly for alternating current apparatus, and the purifying effect of the process extends more nearly throughout its mass than in the case of the necessarily thicker sheets of silicon steel, so that the new product may be made more nearly non-oxygenous than silicon steel, and, of course, much cheaper than silicon steel.

In practising the process any suitable apparatus, especially those fully shown and described in my aforesaid patent may be employed and it is, therefore, unnecessary to here again show and describe the same; a reference to the patent is deemed sufficient. The nature of the raw material, ordinary or commercially pure unalloyed, oxygenous iron, however, prohibits the use of such high temperatures as may be and preferably are employed in the case of silicon steel. With silicon steel I have used temperatures reaching as high as 1325° C. with good effect, but with ordinary or commercially pure unalloyed, oxygenous iron I have found that the practical upper limit is about 1200° C., beyond which it is not necessary to go; nor is it advisable to exceed this temperature on account of the danger of the sticking together of the sheets, which in practice are subjected to the process in packs.

The process is as follows: Ordinary commercial unalloyed, oxygenous iron or so-called commercially pure iron (known as "American ingot iron"), preferably in packs of thin sheets is subjected to a temperature of from 760° C. to 1200° C. either in an evacuated space or in a space through which a reducing gas that is free of carbon, such

as hydrogen, is passed in a continuous stream, for a period of from 2 to 8 hours, depending upon the mass of the material and the temperature employed, the greater 45  
5 mass requiring a longer period and the higher temperature permitting a shorter period. The apparatus shown in my Patent No. 1,110,010, are well adapted for this purpose, and if the vacuum furnace is employed, 10 it should be maintained at a low pressure, at about 2 to 2.5 millimeters of mercury, the lower pressure being preferable. The converted material should be allowed to cool in the furnace to a point where its removal and 15 consequent exposure to the air will not cause any appreciable oxidation.

This process is distinguished from that of heating electrolytic iron in vacuum, which is indicated in the current literature of the 20 art. The material subjected to my process contains among its various impurities notably oxygen, both in chemical combination and occluded. This is true of all ordinary or commercially pure iron, whether it 25 is produced by the open hearth—or Bessemer—or crucible process, and my process has for its object and effects the removal of the impurities and particularly the removal of the oxygen. Electrolytic iron, on the 30 other hand, being a cathode product, contains among its traces of impurities no oxygen; but it contains hydrogen, which is in the nascent state (H) when it is liberated by the electrolysis together with the iron; it 35 is exceedingly active and forms with the iron an alloy which is very hard and brittle. This alloy is broken up and the hydrogen is driven off by heating the material in vacuum.

40 It is conceivable (although the fact has not yet been ascertained) that if in the practice of my process a hydrogen gas ( $H_2$ ) atmosphere is employed, traces of such gas become occluded in the iron; but such gas,

unlike nascent hydrogen, does not alloy with 45 the iron and renders the material neither hard nor brittle; nor has it any other deleterious effect.

What I claim as new and desire to secure by Letters Patent of the United States, is: 50

1. The process of making low hysteresis, high permeability and non-aging magnetic material by annealing, which consists in subjecting commercial unalloyed, oxygenous iron to oxygen removing conditions at a 55 high temperature below that of fusion.

2. The process of making low hysteresis, high permeability and non-aging magnetic material by annealing, which consists in subjecting commercial unalloyed, oxygenous iron to a high temperature below that of fusion under a gas pressure at or below the dissociation pressures of the oxids in the iron for the prevailing temperature. 60

3. The process of making low hysteresis, high permeability and non-aging magnetic material by annealing, which consists in heating commercial unalloyed, oxygenous iron to or above 760° C. but below the fusing 65 temperature in a partial vacuum. 70

4. The process of making low hysteresis, high permeability and non-aging magnetic material by annealing, which consists in heating commercial unalloyed, oxygenous iron to a temperature of 760° C. to 1200° 75 C. under a maintained gas pressure of about 2 to 2.5 millimeters of mercury. 75

5. The process of making low hysteresis, high permeability and non-aging magnetic material by annealing, which consists in subjecting commercial unalloyed, oxygenous iron to oxygen removing conditions at a 80 temperature at least as high as 760° C. but below the temperature of fusion.

In witness whereof, I have hereunto set 85 my hand this 5th day of April, 1916.

WILLIAM E. RUDER.